

## UNITED STATES PATENT OFFICE

1,962,348

## PHOTOGRAPHIC REVERSAL PROCESS

Edwin Ernest Jelley, Wealdstone, England, assignor to Eastman Kodak Company, Rochester, N. Y., a corporation of New York

No Drawing. Application April 2, 1930, Serial No. 441,182. In Great Britain November 13, 1929

11 Claims. (Cl. 95—88)

This invention relates to the production of positive photographic images upon the same support and in the same sensitive layer as that which is exposed in the camera by a reversal process of the kind in which no exposure to actinic light is made after the first development. In such processes sodium sulphide or a compound of formaldehyde and sodium hydrosulphite has hitherto been used to fog or darken the image after the plate or film has been treated in the reversal bath but with the substances hitherto used it has not been possible subsequently to employ the usual photographic developers and as a result the control of the opacity and colour of the final positive image has been considerably restricted.

The object of the present invention is to provide a process by which these disadvantages can be overcome.

According to this invention the film after it has been submitted to the reversal bath is treated with a nucleus-forming agent such as a reducing substance or a selected dye-stuff, in itself well known, prior to redevelopment with any suitable known photographic developer or in conjunction with such developer. As a result the colour and opacity of the final image can be controlled within wide limits during the final developing operation even in the case of very thin emulsions.

Among substances found suitable for use as nucleus-forming or fogging agents prior to or in conjunction with well-known photographic developers, are sodium hydrosulphite, methylene blue, hydrazine and hydrogen peroxide.

The use of hydrazine tends to cause the emulsion to separate from its support during the redevelopment of the film owing to the gas which is then evolved and to counteract this it is therefore necessary for the developer to contain an aldehyde or ketone such for example as formaldehyde acetone or acetaldehyde which combines chemically with the excess of hydrazine and yields an inert compound.

The following are specific examples of how the invention can be carried out.

Example I.—The sensitive plate, film or paper (hereafter referred to as a film) is first exposed in the usual way in the photographic apparatus and fully developed in any known suitable developer such for example as one made up of equal parts of the following solutions:—

## Solution A

|                               | Ounces |
|-------------------------------|--------|
| Hydroquinone                  | 2      |
| Sodium bisulphite             | 3 1/2  |
| Formalin (Commercial)         | 2      |
| Water to make 80 fluid ounces |        |

## Solution B

|                               | Ounces |
|-------------------------------|--------|
| Caustic soda                  | 2 60   |
| Potassium bromide             | 2 1/2  |
| Sodium thiosulphate           | 1      |
| Water to make 80 fluid ounces |        |

After being washed for about a minute the film is bleached in a solution which may be as follows:—

|                               | Parts              |
|-------------------------------|--------------------|
| Potassium bichromate          | 3/4 ounce          |
| Sulphuric acid                | 1 1/4 fluid ounces |
| Water to make 80 fluid ounces | 70                 |

The film is then again washed and immersed in a clearing bath made up as follows:—

|                      | Parts  |
|----------------------|--------|
| Sodium sulphite      | 10     |
| Sodium hydrosulphite | 2 1/2  |
| Water                | 87 1/2 |

After being rinsed, the film is then developed in a caustic hydroquinone developer as above described and subsequently given such washing or other treatment as would be necessary or customary, and is dried in the usual manner.

Example II.—The film is exposed, developed and bleached in the manner above described and after being treated in a 10% aqueous solution of sodium sulphite is immersed in a separate bath containing an aqueous solution of 0.01% methylene blue prior to being redeveloped and treated in the manner already described.

Example III.—Instead of the film being submitted to the action of a fogging or nucleus-forming agent prior to redevelopment, this agent is incorporated in the redeveloping bath. The film after being developed and cleared in a 20% aqueous solution of sodium sulphite is washed and immersed in a caustic hydroquinone developing bath (made up as already described) containing in addition one part of methylene blue to every 1000 parts of developing solution. The addition of this dye-stuff to the developing bath enables the opacity and colour of the image to be controlled within wide limits and eliminates the separate step of treating the film in a bath containing a fogging or nucleus-forming agent prior to redevelopment.

It will be appreciated that the particular solutions stated above are given by way of example only and that considerable modifications may be made in the process within the limits of the invention.

What I claim as my invention and desire to secure by Letters Patent is:—

1. In a process of making positive photographic images by reversal from negative photographic

- images in a light-sensitive element which process comprises rendering the negative image inert and transparent, treating the light-sensitive element by chemical means to render it developable and then developing the sensitive element, the improved step of submitting said element, before development begins, to the action of a solution containing methylene blue as a nucleus-forming agent for the sensitive element.
5. In a process of making positive photographic images by reversal from negative photographic images in a light-sensitive element which process comprises rendering the negative image inert and transparent, treating the light-sensitive element by chemical means to render it developable and then developing the sensitive element, the improved step of submitting said element, before development begins, to the action of a solution containing hydrazine as a nucleus-forming agent for the sensitive element.
10. 2. In a process of making positive photographic images by reversal from negative photographic images in a light-sensitive element which process comprises rendering the negative image inert and transparent, treating the light-sensitive element by chemical means to render it developable and then developing the sensitive element, the improved step of submitting said element, before development begins, to the action of a solution containing hydrazine as a nucleus-forming agent for the sensitive element.
15. 3. A process of making positive photographic images by reversal from negative photographic images in a light-sensitive element which comprises bleaching in an aqueous solution of potassium bichromate and sulphuric acid, treating the light-sensitive element with an aqueous solution of sodium sulphite and sodium hydrosulphite and developing the sensitive element in a caustic hydroquinone developer.
20. 4. A process of making positive photographic images by reversal from negative photographic images in a light-sensitive element which comprises bleaching in an aqueous solution of potassium bichromate and sulphuric acid, clearing and treating the light-sensitive element by immersion respectively in a 10% aqueous solution of sodium sulphite and then in an aqueous solution of 0.01% methylene blue and developing the sensitive element in a caustic hydroquinone developer.
25. 5. A process of making positive photographic images by reversal from negative photographic images in a light-sensitive element which comprises bleaching in an aqueous solution of potassium bichromate and sulphuric acid, immersing the light-sensitive element in an aqueous clearing solution of 20% sodium sulphite and developing in a solution of a caustic hydroquinone developer containing one part of methylene blue to every 1000 parts of developing solution.
30. 6. In a process of making positive photographic images by reversal from negative photographic images in a light-sensitive element which process comprises rendering the negative image inert and transparent, treating the light-sensitive element by chemical means to render it developable and then developing the sensitive element, the
- improved step of submitting said element, before development begins, to the action of a solution containing hydrazine as a nucleus-forming agent for the sensitive element and adding an aldehyde to the solution used in the subsequent developing.
7. In a process of making positive photographic images by reversal from negative photographic images in a light-sensitive element which process comprises rendering the negative image inert and transparent, treating the light-sensitive element by chemical means to render it developable and then developing the sensitive element, the improved step of submitting said element, before development begins, to the action of a solution containing hydrazine as a nucleus-forming agent for the sensitive element and adding a ketone to the solution used in the subsequent developing.
8. In a process for making positive photographic images by reversal from negative photographic images in a light-sensitive element, which process comprises rendering the negative image inert and transparent and then redeveloping the sensitive element, the improved step of rendering the element redevelopable, without reexposure, in developers having ordinary developing properties that comprises submitting the element to a bath including hydrazine.
9. In a process for making positive photographic images by reversal from negative photographic images in a light-sensitive element, which process comprises rendering the negative image inert and transparent and then redeveloping the sensitive element, the improved step of rendering the element redevelopable without reexposure, in developers having ordinary developing properties that comprises submitting the element to a bath including methylene blue.
10. A photographic reversal process comprising the formation of a silver image in a light sensitive, silver halide, emulsion layer, rendering the silver image inert and transparent, treating the remaining silver salts with a bath including a nucleus forming agent and redeveloping the salts with an agent other than the nucleus forming agent.
11. A photographic reversal process comprising the formation of a silver image in a light sensitive, silver halide, emulsion layer, rendering the silver image inert and transparent, treating the remaining silver salts with sodium hydrosulfite to an extent insufficient to reduce the remaining silver salts but sufficient to render them developable, and redeveloping the salts with an agent other than the sodium hydrosulfite.

EDWIN ERNEST JELLEY.

60

135

65

140

70

145

75

150